

April 12, 1932.

J. O. BETTERTON

1,853,537

METAL REFINING

Original Filed Jan. 28, 1930



## UNITED STATES PATENT OFFICE

JESSE O. BETTERTON, OF OMAHA, NEBRASKA, ASSIGNOR TO AMERICAN SMELTING AND REFINING COMPANY, OF NEW YORK, N. Y., A CORPORATION OF NEW JERSEY

**METAL REFINING**

Application filed January 28, 1930, Serial No. 424,134. Renewed September 3, 1931.

The invention relates to refining impure metal mixtures and more particularly to the separation of impurities from lead.

The invention specifically relates to the treatment of the impure skimmings and drosses obtained in the process of refining lead and the selective separation and recovery of certain impurities in said drosses and skimmings such as zinc and bismuth from a lead calcium-zinc-bismuth dross which may be obtained from the refining of impure lead. A portion of the zinc is recovered as a commercial product which may be used cyclicly in the process of refining lead and other by-products are also obtained which may be used in the process cyclicly.

The invention further consists in the new and novel features of operation and the new and original arrangement and combinations 20 of steps in the process hereinafter described and more particularly set forth in the claims.

Although the novel features which are believed to be characteristic of this invention will be particularly pointed out in the claims. 25 appended hereto, the invention itself, as to its objects and advantages, the mode of its operation and the manner of its organization may be better understood by referring to the following description in which a particular 30 commercial embodiment thereof is disclosed. It will be understood however, that the processes and the steps thereof may be modified in various respects without departing from the broad spirit and scope of the invention.

35 The drawing forming a part of this application is a flow sheet illustrating the present process.

In the following description and in the claims the various steps in the process and 40 the details comprising the invention will be identified by specific names for convenience but they are intended to be as generic in their application as the art will permit.

In carrying on the present process a lead 45 dross containing calcium and zinc with or without bismuth and other metals is melted under a chloride slag at a sufficiently high temperature to cause the calcium and a portion of the zinc to form a chloride slag which 50 may be removed from the bath, leaving es-

sentially a lead bath containing zinc and bismuth. The zinc is largely recovered by liquation and retorted to produce metallic zinc. The bath is then treated with chlorine gas to remove the remainder of the zinc as a zinc chloride slag and may then be treated in any suitable manner to recover the other metals therefrom.

The invention is particularly applicable to a lead-calcium-bismuth-zinc dross which 60 is obtained in certain processes for the refining of lead. It may, however, be applied to various other mixtures for the selective separation of the above mentioned metals.

As a specific example of a manner in which 65 this process may be carried out, a bath of lead bullion containing silver, and bismuth and other metals is heated to a temperature of 875° to 900° F., after which zinc is added while suitably stirring the bath to produce 70 the desired reaction. A zinc-silver dross is formed which is skimmed from the bath.

The bath is maintained at a temperature of 650° F., and a calcium-lead alloy added and stirred into the molten metal. A bismuth 75 dross comprising a bismuth-calcium-lead-zinc alloy is removed and treated for the recovery of the zinc contained therein in the manner to be described. The above method of forming the bismuth dross forms no part of the 80 present invention, but is covered in my co-pending application, Serial No. 403,920, filed October 31, 1929, for metal refining.

After this dross is removed chlorine may be added to the bath in sufficient quantities 85 to unite with the calcium and zinc to form slags of zinc chloride and calcium chloride. The slags may be used for treating the above mentioned bismuth dross as outlined below. To treat the lead-calcium-bismuth-zinc dross 90 for the removal of calcium and zinc it is first melted under a slag of calcium chloride and zinc chloride which may be obtained in previous treatment of the lead as above described at a temperature of approximately 1000° F. 95 The resulting slag contains substantially all of the calcium content of the bath as calcium chloride and relatively small amounts of zinc chloride and lead and may be removed and treated for the recovery of the metal values 100

or owing to the low metal content, it may be wasted if desired.

After the removal of the slag the metal is liquated, the liuate portion containing the greater part of the zinc and the bath containing the greater portion of the bismuth. The liquate may be heated in retorts for the production of metallic zinc which may be used in the desilverizing step during the treatment of fresh batches of lead or sold in the market. A small amount of blue powder is formed in the retorts which may be used in any desired manner or further treated to remove the zinc therefrom.

15 The retort metal containing zinc and bismuth is added to the bath which is then treated with chlorine gas to form a zinc chloride slag. This slag contains the remainder of the zinc and may be added to the zinc chloride, 20 calcium chloride slag with which the bismuth dross is treated. The bath will contain the remainder of the bismuth and may be treated in any suitable manner for the recovery thereof.

25 In the above process the lead-bismuth-calcium-zinc dross contains approximately 5% by weight of the bullion treated and is so processed as to allow the recovery of a substantial portion of the zinc as metallic zinc which 30 is in suitable condition for further use in desilverization or for the market. The quantity of zinc chloride slag which is produced in excess of that which can be used for the above described process is reduced to a minimum and the operating time is materially decreased.

Although certain novel features of the invention have been shown and described and are pointed out in the annexed claims, it will 10 be understood that various omissions, substitutions and changes in the forms and details of the device illustrated and in its operation may be made by those skilled in the art without departing from the spirit of the 15 invention.

What is claimed is:

1. The process of treating a lead-calcium-bismuth-zinc dross which comprises melting said dross under a chloride slag capable of 50 selectively chloridizing the calcium to form a calcium chloride slag, removing the larger portion of the zinc from the bath by liquation, removing the remainder of the zinc as a zinc-chloride slag and utilizing said slag for the removal of calcium in the step above described.

2. The process of treating calcium-lead-bismuth-zinc dross which comprises melting said dross under a chloride slag capable of 55 selectively chloridizing the calcium whereby the calcium is removed from the bismuth as a calcium-chloride slag, removing a portion of the zinc by liquation and treating said zinc in retorts whereby metallic zinc is produced.

3. The process of treating a mixture containing bismuth-zinc-calcium-lead which comprises removing calcium as a calcium-chloride slag, partly removing the zinc by liquation and removing the remainder of the zinc as a zinc-chloride slag.

4. The process of treating a mixture of lead, bismuth-calcium and zinc which comprises melting said mixture under a zinc-chloride, calcium-chloride slag at a temperature of approximately 1000° F. whereby the calcium enters the slag, skimming said slag, separating a portion of the zinc from the bath by liquation, treating said portion in retorts to produce blue powder and metallic zinc, returning the retort metal to the bath, treating said bath with chlorine gas to remove the remainder of the zinc as a zinc-chloride slag and treating the bath to recover the bismuth therefrom.

5. The process of treating a lead-calcium-bismuth-zinc dross to remove selectively the calcium and the zinc from the lead and the bismuth, which comprises melting the dross under a slag of zinc chloride and calcium chloride to remove the calcium, then concentrating the zinc in a portion of the bath free from calcium and recovering the zinc therefrom as a metal, then adding chlorine to the bath in quantities sufficient selectively to remove the zinc as zinc chloride without removing the bismuth or lead.

6. The process of treating lead calcium-bismuth-zinc dross to remove selectively the calcium and the zinc from the lead and the bismuth which comprises heating in the presence of zinc chloride to remove selectively calcium and a portion of the zinc as a slag and then treating the residue of the dross with chlorine, to recover the remaining portion of the zinc as zinc chloride for further use cyclically in said process.

7. The process of treating a mixture of lead, bismuth, calcium and zinc which comprises melting said mixture under a zinc-chloride, calcium-chloride slag at a temperature of approximately 1000° F. whereby the calcium enters the slag, skimming said slag, separating a portion of the zinc from the bath by liquation, treating said portion in retorts to produce blue powder and metallic zinc, returning the retort metal to the bath, treating said bath with chlorine gas to remove the remainder of the zinc as a zinc-chloride slag, treating the bath to recover the bismuth therefrom, and returning the zinc-chloride slag to the zinc-chloride, calcium-chloride slag under which the original mixture is melted.

In testimony whereof I have hereunto set my hand.

JESSE O. BETTERTON.